

Dec. 7, 1943.

F. W. LANIGAN ET AL

2,335,865

PACKAGING METHOD

Filed Nov. 17, 1941

Fig. 1



Fig. 2



Fig. 3



Fig. 4



Fig. 5



Fig. 6



Fig. 7



Fig. 8



Inventors:  
Francis W. Lanigan  
Thomas F. Cass Jr.  
By C. H. Seeley

Attty

## UNITED STATES PATENT OFFICE

2,335,865

## PACKAGING METHOD

Francis W. Lanigan, Evanston, and Thomas F. Cass, Jr., Chicago, Ill., assignors of one-half to Container Corporation of America, Chicago, Ill., a corporation of Delaware, and one-half to Dewey and Almy Chemical Company, Cambridge, Mass., a corporation of Massachusetts

Application November 17, 1941, Serial No. 419,468

16 Claims. (Cl. 93—3)

This invention relates to an improved packaging method and more particularly to a packaging method involving paperboard containers having a coating material thereon, such as a coating material adapted to impart moisture vapor-proof properties to paperboard.

Many attempts have been made to devise vapor-tight packages including paperboard containers, but heretofore such packages have either been rather expensive or have not attained the necessary degree of resistance to the passage of gases and vapors, especially moisture vapor. The problem of packaging inexpensively products and commodities which are susceptible to deterioration by change in moisture content, and particularly food products such as prepared cereals, confections, soap flakes, dried fruits, hygroscopic powdered foods, frozen foods and the like, is a very important one which has not heretofore been satisfactorily solved. Such products are now generally packed in combinations of paperboard containers with special wrappers or linings composed of waxed paper, regenerated cellulose or partially depolymerized rubber sheets or similar materials, but each of these packages has one or more disadvantages, such as difficulty of obtaining perfect seals in commercial production, physical instability to temperature changes, and increased labor costs resulting from the necessity of handling such combinations of materials. While attempts have been made to use containers of paperboard coated with a material such as paraffin wax, packages of this type do not have the requisite impermeability, both because paraffin wax is inherently incapable of producing a package having a high degree of resistance of the passage of moisture vapor and because of the difficulty of producing a vapor-tight seal at the package joints. It has also been suggested that paperboard containers already filled be dipped into a bath of paraffin wax or the like, but this has the obvious disadvantage of allowing free transfer of moisture, flavor and odors from the product to the paperboard and vice versa, and as to some products, of necessitating the heating of the contents to an undesirable degree.

We have devised a novel packaging method which is inexpensive and which produces a sealed package affording an unusual degree of protection to the contents thereof. Our invention is particularly adapted to produce substantially moisture vapor-proof packages, but it is not limited thereto, and is applicable to the production of substantially gas-tight or grease-proof packages. It

5 is an object of our invention to provide a packaging method whereby such packages can be inexpensively produced. Another object is to provide a packaging method which can be carried out conveniently and economically on automatic packaging machinery by the manufacturer of the product to be packed therein using a suitable thermoplastic coating material and paperboard containers which can be shipped to such manufacturer in a flat or knocked-down condition. Other objects, uses and advantages of our invention will be apparent from the following detailed description thereof read in conjunction with the drawing, in which:

10 Figure 1 is a diagrammatic flow sheet illustrating the steps comprising the method of our invention in one of its embodiments;

15 Figure 2 is a diagrammatic flow sheet illustrating a modified method according to our invention;

20 Figure 3 shows in perspective a paperboard carton suitable for use in connection with our invention in collapsed or knocked-down form;

25 Figure 4 shows the carton of Figure 3 in expanded or tubular form;

30 Figure 5 shows the carton of Figure 4 as it would appear after the bottom-sealing step and before the filling step;

35 Figure 6 is similar to Figure 5, but brings out the location of the coating applied in accordance with the modification shown in Figure 2;

Figure 7 illustrates the filling step;

Figure 8 shows a filled carton with the top flaps partially closed; and

35 Figure 9 is an enlarged perspective view of one portion of a carton particularly adapted for use in carrying out our method.

40 In one of its broad aspects our invention comprises selecting an empty paperboard container having one open end and one closed end, and overlapping flaps adapted to close the open end, coating at least the interior surfaces of the container and all surfaces of the open flaps with a film of a thermoplastic coating material having good heat-sealing properties, filling the coated containers with a desired product, and closing and heat sealing the coated flaps. While it is not essential, it is extremely desirable that the paperboard containers used be similar to ordinary folding cartons, so that they can be shipped and stored in knocked-down condition. Such cartons are adapted for setting up and bottom sealing with adhesive on conventional automatic equipment and in this form are ready for the coating operation. The flaps at the open

or top end of the carton should be arranged so that they overlap to a very considerable extent and preferably at least the two flaps attached to opposite side walls should be substantially full-sized so as to provide the best possible seal.

The coating operation can be carried out by hand or by any suitable machine, the essential requirements being that the entire container be coated internally and that the open flaps be coated on both sides thereof with a continuous film of a suitable thermoplastic coating material which impregnates the paperboard only enough to adhere firmly thereto. In one embodiment of the invention, the container body is coated externally as well, and this is preferably done by dipping in a molten bath of the coating material, draining and cooling, although flooding or other means can be used. When the outside of the container body is left uncoated, however, flooding is the most suitable procedure for coating the interior surfaces thereof. The thermoplastic coating material should have a softening point such that it will remain in a solid but somewhat pliable condition and not adherent or tacky at any temperature likely to be encountered in storage, shipment or use of the resulting package, and it should have excellent heat-sealing properties which should be superior to those of paraffin wax, for example, so that the container flaps coated with the material and heat-sealed will have substantially no tendency to become detached during handling. Furthermore, the coating material should be of low viscosity and adapted to dipping or flooding operations when in the liquid state, and it preferably has an intermediate "gel" state in which it will flow under heat and pressure. It is obvious, of course, that the coating material should have no characteristic such as odor or taste which would make it unsuitable for direct contact with the product being packaged.

The nature of the thermoplastic coating material will depend, of course, upon the properties which it is desired to impart to the package. It can be of such a nature as to be extremely resistant to the passage of moisture vapor or of inert gas or the like, or to the action of oily or greasy materials, such as peanut butter, for example, or it can have a combination of these properties. In case the product being packed is one which is susceptible to deterioration by change in moisture content, we have found that a particularly suitable thermoplastic coating material is one which is a homogeneous composition including at least 90% of a wax, such as paraffin wax, carnauba wax or beeswax, and in the neighborhood of 7 to 8% of depolymerized rubber. Such compositions having a flow point in the range from about 125° to as high as about 180° F. and especially those having a flow point in the range of 135° to 145° F., have been found to be particularly satisfactory.

Following the coating operation, the cooled coated containers are filled with the product being packed in the usual way. Finally, the open flaps are closed so as to overlap one another and are heat-sealed to provide a completely sealed package, ready for storage or sale.

A diagrammatic flow sheet illustrating a complete packaging operation embodying our invention is shown in Figure 1, and for convenience this will be described in connection with a preferred application thereof to the production of a substantially moisture vapor-proof package. In this instance the paperboard carton used is one of

rectangular cross-section having four integral flaps at each end, all of the side wall flaps being adapted to cover the ends of the carton substantially completely. Such cartons are ordinarily supplied to packers of food products and the like

5 in a flat condition and with one side wall and one end wall secured together by a manufacturer's joint so that it is only necessary to apply pressure to two opposite edges to cause it to assume rectangular shape. Such a carton is illustrated in Figure 3 in substantially flat condition and in Figure 4 in completely expanded condition.

10 The next step is to seal by means of adhesive or the like one end of the carton which will become the bottom end. This operation can be carried out conveniently on conventional automatic machinery capable of folding down the two end wall flaps, applying adhesive to both sides of one of the side wall flaps, folding this over upon the end wall flaps and finally folding down the second side wall flap and holding it in that position until the adhesive has set. The carton then appears as

15 shown in Figure 5.

The next operation is that of coating the 25 bottom-sealed carton with the desired thermoplastic coating material. In this example, the coating material is a homogeneous composition containing about 92.5% of paraffin wax and about 7.5% of rubber which has been depolymerized or 30 modified by prolonged heating, e. g., for 18 hours, at about 300° F. under oxidizing conditions, the vaporized products being continuously withdrawn. This composition has a flow point in the neighborhood of 135° F. and a so-called "gel" state at 35 about 140° to 160° F., and is in a thin liquid state at about 175° to 190° F., the viscosity in the liquid state being of the same order of magnitude as that of the wax used. This material retains its 40 pliable characteristics at temperatures as low as -40° F. so that it will not flake or become dislodged during a freezing operation.

In the modification of Figure 1, the carton is 45 dipped in a bath maintained at the proper temperature, in this instance about 175° to 185° F. It is extremely desirable that the coating material should not penetrate into the paperboard of the 50 carton more than a very small distance sufficient to cause it to adhere thereto at all points, and for this reason the paperboard should not be too porous or have many minute fibres projecting from its surface to act as wicks. The dipping operation itself can be accomplished by any suitable means, the essential feature being that the entire carton, including the flaps thereof, is completely coated on its exterior and interior surfaces. When the carton is withdrawn from the 55 coating bath, it is desirable that the excess coating material should be allowed to drain therefrom in order that the proper film thickness can be obtained. Obviously, it is undesirable that the film should be too thin or inadequate moisture vapor proofing will be obtained and it is also undesirable that this film should be too thick or the coating operation may become uneconomical 60 or the coating may be unevenly deposited so as to produce an undesirable appearance, or it may be more subject to accidental injury or to difficulty in the heat-sealing operation which will be described below. For these reasons, the carton is 65 allowed to remain with its open end down in a draining chamber at a temperature of about 170° to 180° F. for a predetermined period of time. By regulating the temperature of the draining chamber and the time that the carton is within this 70 chamber, it is possible to secure any desired film

weight. Finally, the carton is cooled to solidify the coating material and this is conventionally done by subjecting it to a blast of cool air.

In the modification of Figure 2, the carton is subjected to one or more streams or heavy sprays of the liquid thermoplastic material, which may be directed so as to form a complete film over all of the carton and flap surfaces. As pointed out above, however, it is not essential to the production of a substantially moisture vapor-proof package that the outside of the body portion of the carton be coated, so that only the interior thereof need be subjected to the flooding operation. The top flaps, however, must be completely coated, and this is preferably carried out either as a part of the flooding operation or as a supplementary partial dipping operation. The outside coating may extend from the top flaps merely to their respective score lines, or it may extend a short distance, e. g.,  $\frac{3}{8}$ " to  $\frac{1}{16}$ ", below these score lines as shown in Figure 6. In all of these modifications the cartons are subsequently drained and cooled as hereinabove described.

Many advantages are obtained by coating the carton after the bottom-sealing step, a principal one being that the bottom is thus completely sealed, which would be extremely difficult if it were attempted to seal the bottom end of the carton after it has been coated. Furthermore, in the same operation the manufacturer's joint is made impervious and the edges of the paperboard, for instance, that edge which is on the inside of a carton at the manufacturer's joint, is likewise completely coated so that there will be no opportunity for flavors or odors to pass from the interior of the paperboard to the product to be packed in the carton or for any liquids or gases from the product to be absorbed by the paperboard through this edge.

Since the carton is set up prior to the coating operation, another advantage lies in the fact that, with the exception of the closing of the top flaps, no further folding is required, which might conceivably rupture the continuity of the film of coating material. Any rupture of the film continuity which might occur along the upper horizontal score lines due to the folding of the top flaps is repaired during the proper heat-sealing operation described below.

The coated carton is then ready to be filled with the desired product and this operation can be carried out in a conventional manner, such as illustrated diagrammatically in Figure 7.

The final step is that of top-sealing the filled carton. Since the carton flaps are completely coated with a thermoplastic material having good heat-sealing properties and the property of not impregnating the paperboard except at the surface thereof, it is only necessary to fold the flaps attached to the end walls and then those attached to the side walls, and to apply heat and pressure to the top of the carton sufficient to cause the thermoplastic material to enter its "gel" state and to flow into all of the cracks and crevices between the top flaps and around the edges thereof so that it forms a continuous film sealing the entire top of the carton. In order to insure complete continuity of the coating material film along the upper horizontal scores, where slight ruptures may conceivably occur due to the folding of the top flaps, the heat should be applied over the entire top surface of the carton including the outside edges along the score lines so as to cause the coating material to flow in the vicinity of these scores. As mentioned

above, it is undesirable to have too great a film thickness, since the excess thermoplastic material will only be squeezed from between the flaps and may cause an unsightly result, although a small amount of excess material can be handled if suitable provision is made therefor. Since all of the other points of possible moisture vapor transfer have been completely eliminated by the coating operation, it is apparent that the proper heat-sealing operation completes the continuity of the coating material film and produces a substantially moisture vapor-proof package.

In carrying out our invention as hereinabove described, we prefer to use cartons constructed as shown in Figure 9 having an extension 10 on the glue strip 11 which is adapted to underlie the end wall flap 12. Thus the carton corner which is normally the weakest when the usual cut-back glue strip is used is strengthened, and the continuity of the film of coating material obtained by heat sealing is thus assured.

A modification which can be used involves the application of a special thermoplastic adhesive along the edges of one or more of the top flaps which is not miscible with the thermoplastic coating compound. In this case, the coating material is squeezed out from between those layers of paperboard so coated with such adhesive and the adhesive is thereby caused to adhere directly to the paperboard, causing a paper-to-paper seal, which increases the strength of the bond between the various overlapping flaps.

It will be seen from the above that we have devised a novel and extremely useful packaging method and that various modifications thereof can readily be made by those skilled in the art without departing from the spirit of our invention. We do not desire to be limited, therefore, by the specific embodiments employed in describing our invention, but only by the scope of the appended claims.

We claim:

1. The method of packaging a product which comprises selecting an empty paperboard container having one open end and one closed end, and a plurality of flaps on the side walls thereof adapted to be overlapped to close said open end, coating at least the interior surfaces of said container and all surfaces of said flaps with a film of a thermoplastic coating material which is solid and pliable at normal temperatures and adheres to but does not materially impregnate said paperboard when above its flow point, filling the coated container with said product, closing said flaps, and applying sufficient heat to the closed flaps to cause said material to flow and to form a continuous film completely sealing said flaps, and holding the same in closed position.

2. The method of packaging a product which comprises completely coating an empty paperboard container having one open end and one closed end, and a plurality of flaps on the side walls thereof and integral therewith adapted to be overlapped to close said open end, with a continuous film of a thermoplastic coating material which is solid and pliable at normal temperatures and adheres to but does not materially impregnate said paperboard when above its flow point, filling the coated container with said product, closing said flaps, and applying sufficient heat to the closed flaps to cause said material to flow and to form a continuous film completely sealing said flaps, and holding the same in closed position.

3. The method of packaging a product suscep-

tible to deterioration by change in moisture content which comprises completely coating an empty paperboard container having one open end and one closed end, and a plurality of flaps on the side walls thereof and integral therewith adapted to be overlapped to close said open end, with a continuous film of a thermoplastic coating material substantially impervious to moisture vapor which is solid and pliable at normal temperatures and adheres to but does not materially impregnate said paperboard when above its flow point, filling the coated container with said product and closing and heat-sealing said flaps to form a continuous film holding said flaps in closed position.

4. The method of packaging a product according to claim 3 wherein said thermoplastic coating material is a homogeneous composition including at least 90% of a wax and about 7% to 8% of partially depolymerized rubber.

5. The method of packaging a product which comprises setting up a tubular paperboard carton having integral flaps on the side walls thereof adapted to overlap so as to form closures lying substantially in planes perpendicular to said side walls at both ends thereof, closing and sealing with adhesive the flaps at one end of said carton, coating at least the interior surfaces of said carton and all surfaces of the flaps at the other end of said carton with a continuous film of a thermoplastic coating material which is solid and pliable at normal temperatures and adheres to but does not materially impregnate said paperboard when above its flow point, filling the coated carton with said product, and closing and heat-sealing said last-mentioned flaps to form a continuous film holding said flaps in closed position.

6. The method of packaging a product which comprises setting up a tubular paperboard carton having integral flaps on the side walls thereof adapted to overlap so as to form closures lying substantially in planes perpendicular to said side walls at both ends thereof, closing and sealing with adhesive the flaps at one end of said carton, completely coating said carton with a continuous film of a thermoplastic coating material which is solid and pliable at normal temperatures and adheres to but does not materially impregnate said paperboard when above its flow point, filling the coated carton with said product, and closing and heat sealing the flaps at the other end of said carton to form a continuous film holding said flaps in closed position.

7. The method of packaging a product which comprises dipping an empty paperboard container having one open end and one closed end, and a plurality of flaps on the side walls thereof and integral therewith adapted to be overlapped to close said open end, in a molten bath of a thermoplastic coating material which is solid and pliable at normal temperatures and adheres to but does not materially impregnate said paperboard when above its flow point, whereby both interior and exterior surfaces of said container and flaps come in contact with said material and are coated with a continuous film thereof, removing said container from said bath, cooling said container to solidify the coating material thereon, filling the coated container with said product, and closing and heat-sealing said flaps to form a continuous film holding said flaps in closed position.

8. The method of packaging a product according to claim 7 wherein said thermoplastic coat-

ing material is a homogeneous composition including about 92.5% of paraffin wax and from about 7.5% of rubber which has been depolymerized by prolonged heating, said material having

5 a softening point in the range of 130° to 145° F.

9. The method of packaging a product which comprises selecting an empty paperboard container having one closed end and integral flaps on the side walls thereof adapted to be folded into overlapping relation so as to form a closure lying substantially in a plane perpendicular to said side walls at the other end, coating said container and said flaps internally and externally with a continuous film of a thermoplastic coating material, said material being a solid at normal temperatures and a relatively thin liquid at temperatures well above its flow point, and having a plastic or "gel" state at intermediate temperatures, filling the container so coated with 10 said product, closing said flaps, applying sufficient heat to said flaps to cause the coating material thereon to enter its "gel" state and flow into the adjacent cracks and crevices, and allowing said flaps to cool in closed position, whereby 15 a continuous film of said material is formed completely sealing said flaps, and holding the same in closed position.

10. The method of packaging a product which

comprises setting up a tubular paperboard carton having integral overlapping flaps on the side walls thereof adapted to overlap so as to form closures lying substantially in planes perpendicular to said side walls at both ends thereof, closing and sealing with adhesive the flaps at one 20 end of said carton, coating at least the interior surfaces of said carton and all surfaces of the flaps at the other end of said carton with a continuous film of a normally solid thermoplastic coating material, said material having a plastic

30 state at temperatures up to about 30° F. to 40° F. above its flow point wherein it will flow under light pressure and being a relatively thin liquid at higher temperatures which has the property of impregnating paperboard materially less than

35 40 molten paraffin wax, closing and applying sufficient heat and pressure to said last-mentioned flaps to cause the coating material thereon to flow and to fill the cracks and crevices between and adjacent said flaps, and allowing said flaps 45 to cool in closed position, whereby a continuous film of said material is obtained which completely seals said carton, prevents all contact between the paperboard of said carton and the contents thereof and holds said flaps in closed position.

50 55 11. The method of claim 10 wherein said coating material is a homogeneous composition containing about 92.5% of a wax and about 7.5% of rubber which has been partially depolymerized by heating at a high temperature in the presence 60 of oxygen and with the continuous removal of vaporized decomposition products.

12. The method of packaging a product which comprises setting up a tubular paperboard carton having integral overlapping flaps on the side walls thereof adapted to overlap so as to form closures lying substantially in planes perpendicular to said side walls at both ends thereof, closing and sealing with adhesive the flaps at one end of said carton, dipping said carton in a molten bath of a normally solid thermoplastic coating material, said material having a plastic state at temperatures up to 30°-40° F. above its flow point wherein it will flow under light pressure, and being a relatively thin liquid at higher temperatures which has the property of impregnat-

ing paperboard materially less than molten paraffin wax, removing said carton from said bath, draining excess thermoplastic material therefrom and cooling the drained carton whereby said carton is completely coated with a continuous film of said material, filling the coated carton with said product, closing the flaps at the other end of said carton, applying sufficient heat and pressure to said last-mentioned flaps to cause the coating material thereon to flow and to fill the cracks and crevices between and adjacent said flaps, and allowing said flaps to cool in closed position, whereby a continuous film of said material is obtained which completely seals said carton.

13. The method of claim 12 wherein said coating material is a homogeneous composition containing about 92.5% of a wax and about 7.5% of rubber which has been partially depolymerized by prolonged heating at a high temperature in the neighborhood of 300° F. under oxidizing conditions and with the continuous removal of vaporized decomposition products.

14. The method of claim 12 wherein said coating material is a homogeneous composition containing about 92.5% of paraffin wax and about 7.5% of rubber which has been partially depolymerized by prolonged heating at a high temperature in the neighborhood of 300° F. under oxidizing conditions and with the continuous removal of vaporized decomposition products.

15. The method of sealing one end of a paperboard container having integral flaps on the side walls thereof adapted to be folded into over-

lapping relation so as to form a closure for said end lying substantially in a plane perpendicular to said side walls which comprises coating at least said flaps internally and externally with a continuous film of a thermoplastic coating material, said material being a solid at normal temperatures and a relatively thin liquid at temperatures well above its flow point, and having a plastic or "gel" state at intermediate temperatures, closing said flaps, applying sufficient heat and pressure to said flaps to cause the coating material thereon to enter its "gel" state and to flow into the cracks and crevices between and adjacent said flaps, and allowing said flaps to cool in closed position, whereby a continuous film of said material is formed completely sealing said flaps and holding the same in closed position.

16. The method of sealing at least one end of a paperboard container having a plurality of flaps on the side walls thereof adapted to be overlapped to close said end which comprises coating at least the interior surfaces of said container and all surfaces of said flaps with a film of a thermoplastic coating material which is solid and pliable at normal temperatures and adheres to but does not materially impregnate said paperboard when above its flow point, closing said flaps, and applying sufficient heat to the closed flaps to cause said material to flow and to form a continuous film completely sealing said flaps and holding the same in closed position.

FRANCIS W. LANIGAN,  
THOMAS F. CASS, JR.